

## UNITED STATES PATENT OFFICE.

JUDSON A. DE CEW, OF NEW YORK, N. Y.

## METHOD OF SIZING CELLULOSE FIBERS.

No Drawing.

Application filed December 15, 1925. Serial No. 75,825.

This invention relates to a method of sizing cellulose fibers by means of rosin size emulsions, during the process of paper manufacture.

5 The usual method of sizing paper pulp is to treat the fibers with rosin size and sulphate of alumina in the beating engine where they are mixed with the fibers and sizing precipitates formed in the pulp. Either the size or the alum are added first. 10 The pulp fibers are then discharged into a tank and pumped to a point where they will flow through the Jordan engine and after that they may go direct to the paper machine.

15 It often happens that this method of operation does not properly size the paper, even though the size and alum are of good quality and the reason for this is the fact 20 that some fibers have a poor affinity for rosin emulsions and when the size is added to the stock ahead of the alum, the rosin does not adhere uniformly to the surface of the fibers by adsorption and when it is precipitated 25 by the alum it is in such a form that it drains from the fibers on the wire and is lost.

In order to change the character of such 30 a cellulose so that it will adsorb the rosin from suspension or from colloidal solution, it is necessary to first treat the cellulose with sulphate of alumina and then later add the size emulsion so that it is precipitated on the fibers by the acidity within the fibers.

35 When this process is carried out in the beating engine however, this reaction does not take place because the beater mixes the size with the fibers so slowly that the size is coagulated by the acid water surrounding the fibers and not by the acid fibers themselves so that no final improvement is obtained by using this method.

I have discovered, however, that the size can be precipitated directly upon the fibers if the mixing action is very rapid so that the size emulsions cover the fibers at the 45 time that they are precipitated and I obtain this result by the following method of operation:

I first treat the fibers in the beating engine with the required amount of sulphate 50 of alumina and allow them to remain in contact with the alum solution long enough for the fibers to adsorb a portion of the sulphate of alumina. The stock is then discharged from the beater and pumped to the Jordan 55 and as the fibers pass into the Jordan engine a continuous stream of sizing emulsions passes into the Jordan along with the stock.

In this machine the mixing action is so 60 rapid that the size is uniformly spread over the fibers at the time of coagulation and a part of the coagulation is caused by the acidity already in the fibers.

In this way the pulp fibers are better sized 65 than they would be if the sizing ingredients were all put into the beater where the mixing is slow and coagulation is rapid.

What I claim as my invention is:—

1. A method of sizing paper pulp which 70 consists in a continuous mixing treatment of rosin size emulsions and paper making fibers, within the Jordan engine, the fibers already having been made astringent by previous treatment with sulphate of alumina. 75

2. A method of sizing paper pulp, which consists in treating the fibers while in the beater with sulphate of alumina and adding a stream of size emulsion to the fibers as 80 they are entering the Jordan engine.

In testimony whereof, I affix my signature.  
JUDSON A. DE CEW.